# EUROPEAN PATENT SPECIFICATION

(11) **EP 1 760 137 B1**
(45) Date of publication and mention of the grant of the patent: **04.04.2012**
(21) Application number: 06254370.7
(22) Date of filing: 21.08.2006
(51) Int. Cl.: C10M 159/16, C10N 10/02, C10N 10/04, C10N 30/04, C10N 40/25

(54) **The use of a Mannich condenstation product as an anti-wear additive agent in a low sulfur, low sulfated ash and low phosphorus lubricating oil composition for heavy duty diesel engines**
Die Verwendung von Mannichprodukte als Verschleissschutzadditiv in Schmierölzusammensetzung mit niedrigem Gehalt an Schwefel, Sulfatasche und Phosphor für Hochleistungsdieselmotoren
L'Utilisation d'un produit Mannich comme additif anti-usure pour huile lubrifiant à faible teneur en soufre, en cendres sulfatées et en phosphore pour moteurs diesel de grande puissance

(30) Priority: 31.08.2005 US 218208
(43) Date of publication of application: 07.03.2007
(73) Proprietor: Chevron Oronite Technology B.V., 3196 KD Vondelingenplaat, Rotterdam (NL)
(72) Inventor: Kleijwegt, Peter, 3274 LK Heinenoord (NL)
(74) Representative: Nash, David Allan

(56) References cited:
- EP-A2- 1 167 497
- US-A- 3 912 707
- US-A- 4 088 586
- US-A- 4 131 551
- US-A- 5 370 805

## Description

The present invention is directed to the use of a metal salt of a Mannich condensation product as an anti-wear agent in a low sulfur, low sulfated ash and low phosphorus lubricating oil composition for low emission heavy duty diesel engines comprising a major amount of an oil of lubricating viscosity. The metal salt of a Mannich condensation product produced is use in amount of at least 2 weight percent based on the total weight of the lubricating oil.

Heavy duty diesel internal combustion engines mounted on motor-driven vehicles, constructions machines and power generators are generally driven using gas oil or heavy oil (which is a fuel having a sulfur content of approxi-mately 0.05 wt.% or more). Most lubricating oils for the diesel engines have a sulfur content of approximately 0.3 to 0.7 weight percent, a sulfated ash content of approximately 1.3 to 2.0 weight percent, and a phosphorus content of approximately 0.1 to 0.13 weight percent.

In order to reduce air pollution, vehicle manufacturers and petroleum companies are interested in developing lubricating oil systems that have low emissions and better fuel economy for heavy duty diesel engines. Environmental pollution caused by emissions from diesel engines may comprise particulates and carbon oxides, sulfur oxides and nitrogen oxides. Diesel engine manufacturers have started to equip diesel engines with exhaust after-treatment devices containing particulate filters, oxidation catalysts and reduction catalysts to obviate environmental problems.
Both the fuel and the lubricating oil used to lubricate diesel engines contribute to particulates and oxides found in emissions from diesel engines. Conventionally used anti-wear agents and anti-oxidants, such as zinc di-alkyl di-thiophosphates, contribute to reduction in the activity of the oxidation catalysts, thus, reduction in phosphorus levels reduces the deactivation of the catalysts used in exhaust after-treatment devices. The zinc in zinc di-alkyl di-thiophosphates may also contribute to sulfated ash which may clog the particulate filters. Therefore, there is a need to decrease the phosphorus and zinc content in the lubricating oil to protect the oxidation catalysts from deterioration and to prevent the clogging of the particulate filters.

Another major concern is sulfated ash derived from the salts of alkali and alkaline earth metal detergent additives in lubricating oil. The non-combustible ash deposits in diesel engines become trapped in the channels of diesel engine exhaust gas particulate filters. Conventional lubricating oils used in diesel engines are also high in sulfur content, which originates in the additive components and the base oil. Sulfur in diesel fuels is converted to sulfuric acid and sulfates which emigrate to the exhaust gas cleaning devices and contribute to the particulates that clog the particulate filters in heavy duty diesel engine vehicles equipped with them. Sulfuric acid may also indirectly contribute to clogging the particulate filters by wetting the particulates, thus adding to their mass. The sulfuric acid and the sulfates also poison the oxidation catalysts in the exhaust gas cleaning devices which may also result in failure to meet emission requirements. Thus, for continued functioning of these particulate traps and oxidation catalysts, it is essential that the sulfur and sulfated ash content in the lubricating oil is lowered considerably compared to the conventional diesel engine lubricating oils.

A number of patents and patent applications have discussed methods for reducing particulate emissions and low sulfur, low sulfated ash and low phosphorus lubricating oil compositions, but none have disclosed a low sulfur, low sulfated ash and low phosphorus lubricating oil composition comprising an anti-wear additive composition comprising a Mannich condensation product for a low emission diesel engine, wherein the anti-wear additive composition is also providing detergency.

Canadian Patent No. 810120 discloses a lubricating oil composition comprising the low sulfated ash and low viscosity reaction product obtained by the neutralization with an alkaline earth metal oxide or hydroxide of a sulfurized alkylphenol in admixture with a Mannich base reacted with carbon dioxide.

U. S. Patent No. 4,089,791 discloses a lubricating oil composition comprising a major portion of a mineral lubricating oil and minor amounts of an overbased alkaline earth metal compound, of a tri-alkanolamine and a zinc di-hydrocarbyl di-thiophosphate for reduction of bearing weight loss in an internal combustion engine, while retaining the low ash and rust inhibition properties.

U. S. Patent No. 4,330,420 discloses low ash, low phosphorus motor oils having improved oxidation stability as a result of the addition of synergistic amounts of a di-alkyl di-phenylamine anti-oxidant and of a sulfurized polyolefin. The synergism between the two additives compensates for the decreased amount of phosphorus in the form of zinc di-thiophosphate such that the oils retain an SE quality rating.

U. S. Patent No. 5,102,566 discloses a low sulfated ash lubricating oil composition which comprises a base oil, at least about 2 weight percent of an ashless nitrogen- or ester-containing dispersant, an oil-soluble antioxidant material, and an oil soluble di-hydrocarbyl di-thiophosphate anti-wear material, and which has a total sulfated ash level of 0.01 to 0.6 weight percent and a weight ratio of total sulfated ash and the dispersant in the range of 0.01:1 to 0.2:2.

U. S. Patent No. 5,490,945 discloses lubricating oil compositions and concentrates containing alkali metal overbased salts of carboxylic acids and either magnesium overbased salts of acidic compounds having a metal ratio of at least 3 provided that the lubricating composition is free of calcium overbased salts of acidic compounds having a metal ratio greater than 3 provided that the lubricating composition is free of magnesium overbased salts having a metal ratio greater than 3.

U. S. Patent No. 6,114,288 discloses a lubricating oil composition for internal combustion engines having a high temperature shear viscosity of from 2.1 to less than 2.9 mPas, wherein the lubricating base oil comprises (1) a zinc di-alkyl di-thiophosphate, (2) a metallic detergent chosen from calcium alkylsalicylate and a mixture of calcium alkyl and magnesium alkylsalicylate and optionally (3) friction modifier. The lubricating oil composition overcomes the problems of scuffing and the wear resistance of moving parts under severe lubrication conditions.

U. S. Patent No. 6,159,911 discloses a diesel engine oil composition containing a lube oil base and one or more metallic detergents-dispersants selected from among a perbasic alkaline earth metal sulfonate, phenolate and salicylate. The total phosphorus content of the composition is suppressed to 100 parts per million by weight or less, to thereby provide diesel engine oil compositions having oxidation stability and wear resistance.

U. S. Patent No. 6,162,770 discloses an un-sulfurized, alkali metal-free, detergent-dispersant composition having from about 40% to 60% alkylphenol, from 10% to 40% alkaline earth alkylphenol, and from 20% to 40% alkaline earth single aromatic-ring alkylsalicylate. This composition may have an alkaline earth double aromatic-ring salicylates as long as the mole ratio of single-ring alkylsalicylate to double aromatic ring alkylsalicylate is at least 8:1.

U. S. Patent No. 6,277,794 discloses a marine diesel lubricant composition having a TBN of at least 10 and preferably a VI of at least 90, comprise a major amount of oil of lubricating viscosity, and admixed therewith, minor amounts of an ashless anti-wear additive and a metal detergent in the form of (i) an overbased metal detergent having a TBN of at least 300, more preferably at least 400, and comprising a surfactant system derived from at least two surfactants, and/or (ii) a metal detergent other than (i); provided that, if detergent (ii) is present, the composition does not contain a minor amount of an extreme pressure additive, being up to 5.0 mass percent on the total mass of the composition.

U. S. Patent Nos. 6,331,510 and 6,610,637 disclose a lubricant containing (a) a synthetic base oil composition having an overall kinematic viscosity of at least about 4.8X10⁻⁶ m²/s (4.8 cSt) at 100°C and a viscosity index of at least 110; (b) a dispersant-viscosity modifier; and (c) a sulfur-free functionalized hydrocarbyl-substituted phenol detergent provides improved valve train wear, with longer drain intervals, to heavy duty diesel engines.

U. S. Patent No. 6,376,434 discloses a lube composition which is suitably used for diesel engines which exhaust large amounts of sulfur dioxides. The composition exhibits corrosion/wear preventive properties against sulfur dioxides. The lube composition includes a lube base oil, a component (A) which is a compound selected from a group consisting of overbased sulfonates of alkaline earth metal, overbased phenates of alkaline earth metals and overbased salicylates of alkaline earth metals, and a component (B) which is a bis-type succinimide compound.

U. S. Patent No. 6,730,638 discloses a lubricating oil for internal combustion engines especially useful with fuels having less than 350 parts per million sulfur comprises a lubricating oil basestock, a boron containing ashless dispersant, a molybdenum containing friction reduction agent, a metal type detergent and zinc di-thiophosphate.

U. S. Patent No. 6,784,143 discloses the use of a minor amount of a detergent composition comprising one or more metal detergents which comprises metal salts of organic acids , wherein the detergent composition comprises more than 50 mole percent, based on the moles of the metal salts of organic acids in the detergent composition, of: (I) a metal salt of an aromatic carboxylic acid, or (II) a metal salt of a phenol, or (III) both a metal salt of an aromatic carboxylic acid and a metal salt of a phenol, in a lubricating oil composition for improving oxidation resistance of the lubricating oil composition, wherein the amount of phosphorus and sulfur in the oil composition is less than 0.09 mass % and at the most 0.5 mass % respectively, based on the mass of the oil composition. It has also been found that a detergent composition comprising more than 50 mole % of a metal salt of an aromatic carboxylic acid improves the reduction in wear in an engine.

European Patent Application No. 01201752.1 (Publication No. EP 1 256 619 A1) deemed withdrawn as of March 5, 2005, and U.S. Patent Application NO. 10/142,513 (Publication No. US 2003/0096716 A1) disclose a lubricating oil composition comprising: (A) an oil.of lubricating viscosity, in a major amount and added thereto: (B) a detergent composition comprising one or more metal detergents which comprises metal salts or organic acids, in a minor amount, wherein the detergent composition comprises more than 50 mole percent of a metal salt of an aromatic carboxylic acid, based on the moles of the metal salts of organic acids in the detergent composition, and (C) one or more co-additives, in a minor amount; wherein the total amounts of phosphorus and sulfur derived from (B) or (C) or both (B) and (C) are less than 0.1 mass p% of phosphorus and at the most 0.5 mass % of sulfur, based on the mass of the oil composition. It has been found that a detergent composition comprising more than 50 mole % of a metal salt of an aromatic carboxylic acid improves the reduction in wear in an engine.

U.S. Patent Application No. 10/430,594 (Publication No. US 2003/0216266 A1) discloses a lubricating oil composition employable in combination with a low sulfur content fuel oil is preferably composed of a base oil having a sulfur content of at most 0.2 weight percent , an ashless dispersant comprising an alkenyl- or alkyl-succinimide or derivative thereof, a metal-containing detergent containing an organic acid metal salt, a zinc di-alkyl di-thiophosphate, thiophosphate, a zinc di-alkylaryl di-thiophosphate, and an oxidation inhibitor selected from a group consisting of a phenol compound, an amine compound, and a molybdenum-containing compound, wherein a ratio of the phosphorus content of the zinc di-alkyl di-thiophosphate to the phosphorus content of the zinc di-alkylaryl di-thiophosphate is in the range of 20:1 to 2:1.

International Publication No. WO 2004/046283 A1 discloses the use of lubricating oils with low sulfur content in combination with a low sulfur fuel to reduce particulate emissions of a diesel engine equipped with a particulate trap.

EP-A-1167 497 discloses a lubricating oil composition having a low P content of 0.01 to 0.1 wt.%, and a sulfated ash of 0.1 to 1 wt.%, which is composed of a) a major amount of mineral base oil having a low S content of at most 0.1 wt.%; b) an ashless alkenyl or alkyl-succinimide dispersant; c) a metal-containing detergent (non-sulfurized alkali metal or alkaline earth metal salt of an alkylsalicylic acid and/or non-sulfurized alkali metal or alkaline earth metal salt of an alkylphenol derivative having a Mannich base structure); d) Zn-DTP; e) an oxidation inhibitor (phenol compound and/or amine compound) and wherein the sulfur content is 0.01 to 0.3 wt %. The lubricating oil composition shows good high temperature detergency notwithstanding its low S, P, and sulfated ash content, and is favourably employable in diesel engines using fuel of an extremely low sulfur content.

### SUMMARY OF THE INVENTION

The present invention is directed to the use of a metal salt of a Mannich condensation product as an anti-wear agent in a low sulfur, low sulfated ash and low phosphorus lubricating oil composition for low emission heavy duty diesel engines, wherein the metal salt of a Mannich condensation product is used in an amount of at least 2 weight percent based on the total weight of the lubricating oil composition, and wherein:
(a) the sulfur content of the lubricating oil composition is in the range of 0.0 weight percent to 0.4 weight percent based on the total weight of the lubricating oil;
(b) the sulfated ash content of the lubricating oil composition is in the range of 0.2 weight percent to 4.0 weight percent based on the total weight of the lubricating oil; and
(c) the phosphorus content of the lubricating oil composition is in the range of 0.005 weight percent to 0.06 weight percent based on the total weight of the lubricating oil.

The Mannich condensation product employed as an anti-wear agent surprisingly shows anti-wear performance while maintaining good detergency.

Preferably the concentration of the Mannich condensation product is from 2 weight percent to 12 weight percent based on the total weight of the lubricating oil composition. More preferably the concentration of the Mannich condensation product is preferably from 3 weight percent to 9 weight percent based on the total weight of the lubricating oil composition, and most preferably the concentration of the Mannich condensation product is preferably from 4 weight percent to 7 weight percent based on the total weight of the lubricating oil composition.

The Mannich condensation product used as an anti-wear additive composition in the lubricating oil may be prepared from a formaldehyde or an aldehyde having one carbon atom to 10 carbon atoms, a nitrogen base selected from ammonia, a lower alkyl amine, a polyamine and mixtures thereof, and an alkylphenol.

The alkyl group on the alkylphenol employed to prepare the Mannich condensation product may be a linear chain or a branched chain alkyl group. Preferably the alkyl group on the alkylphenol employed to prepare the Mannich condensation product is a branched chain alkyl group.

Preferably the branched chain alkyl group on the alkylphenol employed to prepare the Mannich condensation product has from 4 carbon atoms to 60 carbon atoms. More preferably the alkyl group on the alkylphenol has from 6 carbon atoms to 40 carbon atoms. Most preferably the alkyl group on the alkylphenol has from 8 carbon atoms to 20 carbon atoms.

The aldehyde useful for the preparation of the Mannich condensation product is an aldehyde having one carbon atom to about 10 carbon atoms. Preferably the aldehyde is formaldehyde, and more preferably it is paraformaldehyde.

The nitrogen base is selected from ammonia, a lower alkyl amine, wherein the alkyl group has one carbon atom to 10 carbon atoms, a poly amine having 2 to 12 amine nitrogen atoms and 2 to 40 carbon atoms.

Preferably the nitrogen base for the preparation of the Mannich condensation product is a lower alkyl amine, wherein the alkyl group has one carbon atom to 10 carbon atoms. The lower alkyl amine is an alkyl mono-amine, such as mono-methyl amine, mono-ethyl amine, mono-propyl amine, monobutyl amine and mono-pentyl amine. More preferably the alkyl mono-amine is mono-methyl amine.

The polyamine useful for the preparation of the Mannich condensation product includes mono-alkylene polyamines and polyalkylene polyamines.

In a preferred embodiment of the present invention, the Mannich condensation product is prepared from an alkylphenol wherein the alkyl group on the alkylphenol is a branched chain alkyl group having from 8 carbon atoms to 20 carbon atoms, paraformaldehyde and mono-methyl amine.

The metal in the metal salt of a Mannich condensation product may be an alkali metal or an alkaline earth metal. Preferably the metal is an alkaline earth metal, and more preferably the alkaline earth metal is calcium.

The sulfur content of the lubricating oil composition is in the range of 0.0 weight percent to 0.4 weight percent based on the total weight of the lubricating oil. More preferably the sulfur content of the lubricating oil composition is in the range of 0.05 weight percent to 0.3 weight percent based on the total weight of the lubricating oil. Most preferably the sulfur content of the lubricating oil composition is in the range of 0.1 weight percent to 0.2 weight percent based on the total weight of the lubricating oil.

The sulfated ash content of the lubricating oil composition is in the range of 0.2 weight percent to 4.0 weight on the total weight of the lubricating oil. More preferably the sulfated ash content of the lubricating oil composition is in the range of 0.3 weight percent to 2.0 weight percent based on the total weight of the lubricating oil. Most preferably the sulfated ash content of the lubricating oil composition is in the range of 0.5 weight percent to 1.2 weight percent based on the total weight of the lubricating oil.

The phosphorus content of the lubricating oil composition is in the range of 0.005 weight percent to 0.06 weight percent based on the total weight of the lubricating oil. More preferably the phosphorus content of the lubricating oil composition is in the range of 0.015 weight percent to 0.05 weight percent based on the total weight of the lubricating oil. Most preferably the phosphorus content of the lubricating oil composition is in the range of 0.03 weight percent to 0.04 weight percent based on the total weight of the lubricating oil.

The above lubricating oil composition may further comprise one or more lubricating oil additives selected from detergents, dispersants, anti-oxidants, viscosity index improvers, corrosion inhibitors, anti-wear agents, friction modifiers, pour point depressants and foam inhibitors.

Preferably the above lubricating oil composition further comprises one or more dispersants. More preferably the dispersants are ashless dispersants. Most preferably the ashless dispersants are derivatives of succinic anhydride. The lubricating oil composition may also contain viscosity index improvers such as polyalkyl methacrylates, ethylene-propylene copolymers, styrene-butadiene copolymers and polyisoprene.

Corrosion inhibitors and anti-oxidants optionally contemplated for use in the lubricating oil are metal di-alkyl di-thiophosphates and derivatives of di-phenyl amine.

Metal di-alkyl di-thiophosphates may also be included in the lubricating oil composition to control wear. However, it may be advantageous to control the amount of these additives because their metal contributes to sulfated ash in the lubricating oil and the phosphorus will be harmful to the exhaust gas oxidation catalysts. Examples of metal di-alkyl di-thiophosphates are zinc and molybdenum salts of di-alkyl di-thiophosphates.

Typically, friction modifiers are used to impart the proper friction characteristics to the lubricating oil composition. Useful friction modifiers are fatty acid esters and amides and molybdenum compounds, such as amine-molybdenum complex compound and molybdenum di-thiocarbamates. However, it should be noted that the addition of molybdenum di-thiocarbamates will further contribute sulfur to the lubricating oil composition and sulfated ash to the exhaust system.

Pour point depressants lower the temperature at which the fluid will flow or can be poured. Additives that optimize the low temperature fluidity of the lubricating oil are various copolymers, such as polymethacrylates.

Useful foam inhibitors are of the polysiloxane type.

Described herein is a low sulfur, low sulfated ash and low phosphorus lubricating oil concentrate for low emission heavy duty diesel engines comprising:
(a) 10 weight percent to 90 weight percent of an oil of lubricating viscosity based on the total weight of the lubricating oil concentrate; and
(b) at least 2 weight percent of an anti-wear additive composition comprising a metal salt of a Mannich condensation product based on the total weight of the lubricating oil composition.

Also described is a method for lubricating low emission heavy duty diesel engines, which comprises lubricating with a low sulfur, low sulfated ash and low phosphorus lubricating oil composition comprising:
(a) a major amount of an oil of lubricating viscosity; and
(b) at least 2 weight percent of an anti-wear additive composition comprising a metal salt of a Mannich condensation product based on the total weight of the lubricating oil composition.

### DETAILED DISCRIPTION OF THE INVENTION

### DEFINITIONS

As used herein, the following terms have the following meanings unless expressly stated to the contrary:

The term "alkali metal" as used herein refers to Group I metals of the Periodic Table, such as sodium, potassium and lithium.

The term "alkaline earth metal" as used herein refers to Group II metals of the Periodic Table, such as calcium and magnesium.

The term "detergents" as used herein refers to additives designed to hold the acid-neutralizing compounds in solution in the oil. They are usually alkaline and react with the strong acids (sulfuric and nitric) which form during the combustion of the fuel and which would cause corrosion to the engine parts if left unchecked. Suitable detergents for use in the present invention are alkyl sulfonates, alkyl phenates and Mannich base condensation products. Numerous detergents are commercially readily available.

The term "dispersants" as used herein refers to additives that keep soot and combustion products in suspension in the body of the oil charge and therefore prevent deposition as sludge or lacquer. Typically, the ashless dispersants are nitrogen-containing dispersants formed by reacting alkenyl succinic acid anhydride with an amine. Examples of such dispersants are alkenyl succinimides and succinamides. These dispersants can be further modified by reaction with, for example, boron or ethylene carbonate. Ester-based ashless dispersants derived from long chain hydrocarbon-substituted carboxylic acids and hydroxy compounds may also be employed. Preferred ashless dispersants are those derived from polyisobutenyl succinic anhydride. Dispersancy may also be controlled by dispersant viscosity modifiers, such as polymethacrylates, alkylmethacrylate styrene copolymers, polyalkylmethacrylates and olefin copolymers. A large number of dispersants are commercially available. The term "overbased" as used herein refers to alkaline earth metal alkylphenols, alkyl salicylates and alkyl sulfonates in which the ratio of the number of equivalents of an alkaline earth metal to the number of equivalents of the organic moiety is greater than 1. Low overbased refers to alkaline earth metal alkylphenols, alkyl salicylates and alkyl sulfonates having a Total Base Number (TBN) greater than 1 and less than 20, medium overbased refers to alkaline earth metal alkylphenols, alkyl salicylates and alkyl sulfonates having a TBN greater than 20 and less than 200. High overbased refers to alkaline earth metal alkylphenols, alkyl salicylates and alkyl sulfonates having a TBN greater than 200.

The term "sulfated ash" as used herein refers to the non-combustible residue resulting from detergents and metallic additives in lubricating oil. Sulfated ash was determined using ASTM Test D874.

The term "Total Base Number" or "TBN" as used herein refers to the amount of base equivalent to milligrams of KOH in one gram of sample. Thus, higher TBN numbers reflect more alkaline products, and therefore a greater alkalinity. TBN was determined using ASTM D 2896 test.

Unless otherwise specified, all percentages are in weight percent.

### LUBRICATING OIL COMPOSITION

It has been discovered that the a low sulfur, low sulfated ash and low phosphorus lubricating oil composition comprising an anti-wear additive composition comprising a metal salt of a Mannich condensation product provides good wear control when used for low emission heavy duty diesel engines. Wear control in conventional lubricating oil compositions is achieved by the addition of metal salts of di-alkyl di-thiophosphates, for example zinc di-alkyl di-thiophosphates, however, the metal in these anti-wear additives contributes to an increase in sulfated ash in the lubricating oil and the phosphorus causes inactivation of oxidation catalysts used in exhaust after-treatment devices. The anti-wear additive composition employed in the lubrication oil composition provides good wear control without contributing to an increase in sulfur and sulfated ash, and because it does not contain any phosphorus, it does not inactivate the oxidation catalysts.

The lubricating oil composition may be prepared by simple blending or mixing of the compounds described in more detail below. These compounds may also be preblended as a concentrate or package with various other additives in appropriate ratios to facilitate blending of a lubricating oil composition containing the desired concentration of additives.

### Oil of Lubricating Viscosity

Oil of lubricating viscosity, or base oil as used herein refer to lubricating oils which may be mineral oil or synthetic oils of lubricating viscosity and preferably useful in the crankcase of an internal combustion engine. Crankcase lubricating oils ordinarily have a viscosity of about 1300 centistokes at -17.8°C to 22.7 centistokes at 98.9°C. The lubricating oils may be derived from synthetic or natural sources. Mineral oil for use as the base oil in this invention includes paraffinic, naphthenic and other oils that are ordinarily used in lubricating oil compositions. Synthetic oils include hydrocarbon synthetic oils and synthetic esters. Useful synthetic hydrocarbon oils include liquid polymers of alpha-olefins having the proper viscosity. Especially useful are the hydrogenated liquid oligomers of C₆ to C₁₂ alpha-olefins such as 1-decene trimer. Similarly, alkyl benzenes of proper viscosity, such as didodecyl benzene, may be used. Useful synthetic esters include the esters of both mono-carboxylic acids and polycarboxylic acids as well as mono-hydroxy alkanols and polyols. Typical examples are didodecyl adipate, pentaerthritol tetracapoate, di-2-ethylhexyl adipate, di-laurylsebacate and the like. Complex esters prepared from mixtures of mono- and di-carboxylic acid and mono- and di-hydroxy alkanols can also be used. Blends of hydrocarbon oils and synthetic oils may also be used. For example, blends of 10 weight percent to 25 weight percent hydrogenated 1-decene trimer with 75 weight percent to 90 weight percent 683 centistokes at 37.8°C mineral oil gives an excellent oil base. Fischer-Tropsch derived base oils may also be employed in the lubricating oil composition of the present invention.

It is further contemplated that the oil of lubricating viscosity employed for preparing the lubricating oil composition is a low sulfur base oil. Use of a low sulfur base oil assists in obtaining a lubricating oil composition which is ultra low in sulfur content. Sulfur content of base oils is well known by persons skilled in the art, thus, selection of a low sulfur base oil may be conveniently made for the purpose of the present invention.

### Anti-wear Additives

### Metal salt of Mannich condensation product

The Mannich condensation product may be prepared using an alkylphenol, an aldehyde and a nitrogen base selected from ammonia, a lower amine, a polyamine and mixtures thereof.

The alkyl group on the alkylphenol employed to prepare the Mannich condensation product is a linear chain or a branched chain alkyl group. Preferably the alkyl group on the alkylphenol employed to prepare the Mannich condensation product is a branched chain alkyl group.

The alkyl group on the alkylphenol used for the preparation of the Mannich condensation product may be a branched chain alkyl group containing from 4 carbon atoms to 60 carbon atoms or a linear chain alkyl group containing from 6 carbon atoms to 60 carbon atoms. Preferably the alkyl group on the alkylphenol is a branched chain alkyl group containing from 8 carbon atoms to 20 carbon atoms. Preferably the alkyl group is attached to the alkylphenol moiety at the ortho-position or the para-position to the hydroxyl group.

More preferably the ratio of the attachment of the alkyl group in the ortho-position to para-position is 20:80 based on the total alkylphenol, and most preferably the ratio of the attachment of the alkyl group in the ortho-position to para-position is 5:95 based on the total alkylphenol.

The aldehyde useful for the preparation of the Mannich condensation product is an aldehyde having one carbon atom to 10 carbon atoms. Preferably the aldehyde is formaldehyde, and more preferably it is paraformaldehyde.

The nitrogen base is selected from ammonia, a lower alkyl amine, wherein the alkyl group has one carbon atom to 10 carbon atoms, a polyamine having 2 to 12 amine nitrogen atoms and 2 to 40 carbon atoms.

Preferably the nitrogen base for the preparation of the Mannich condensation product is a lower alkyl amine, wherein the alkyl group has one carbon atom to 10 carbon atoms. The lower alkyl amine is an alkyl mono-amine, such as mono-methyl amine, mono-ethyl amine, mono-propyl amine, monobutyl amine and mono-pentyl amine. More preferably the alkyl mono-amine is mono-methyl amine.

The polyamines useful for preparation of the Mannich condensation product employed as an anti-wear additive in the present invention include mono-alkylene polyamines and polyalkylene polyamines. Examples of mono-alkyl polyamines include ethylene di-amine, ethylene tri-amines and ethylene tetra-amines, propylene di-amine and propylene tri-amine. Examples of polyalkylene polyamines include di-ethylene di-amine, di-(trimethylene) tri-amine, di-propylene tri-amines and tri-ethylene tetra-amine.

Metal salts of the Mannich condensation product employed in the lubricating oil composition may be prepared by any method known to a person skilled in the art. Generally, the Mannich condensation product is prepared by reaction of the alkylphenol, formaldehyde and mono-alkyl amine in the presence of a metal hydroxide and a diluent.

The preparation of Mannich condensation product is well known to persons skilled in the art. The Mannich condensation product may be prepared using an alkylphenol, an aldehyde and an amine by any method known to a person skilled in the art. For example, the Mannich condensation product may be prepared as described in U.S. Patent 5,370,805.

The metal salt of the Mannich condensation product may be prepared by any well know process using a metal oxide, metal hydroxide or a metal alkoxides. The metal may be an alkali metal or an alkaline earth metal. Preferably the metal is an alkaline earth metal, and more preferably the alkaline earth metal is calcium.

### Other Additives

The lubricating oil composition may also typically contain, in addition to the detergent composition, other additives used to impart desirable properties to the lubricating oil composition. Thus, the lubricating oil may contain one or more of additives, such as, dispersants, anti-oxidants, viscosity index improvers, corrosion inhibitors, anti-wear agents, friction modifiers, pour point depressants and foam inhibitors.

For best overall results in terms of affording the properties desired in a conventional lubricating oil composition for a heavy duty diesel engine lubricating oil, the lubricating oil contains a compatible combination of additives of each of the above classes of additives in effective amounts as well as the detergent composition in the amount needed to provide the desired neutralization capacity.

### Low, Medium and High Overbased Metal Detergents

Small quantities of low or medium overbased metal detergents may optionally be employed in the lubricating oil composition. Examples of the low and medium overbased metal detergents are low or medium overbased sulfonic acids, salicylic acids, carboxylic acids, or phenols or Mannich condensation products of alkylphenols, aldehydes and amines. These detergents may be alkali metal detergents or alkaline metal detergents. Preferably they are alkaline earth metal detergents and more preferably they are calcium detergents. The TBN of these detergents is greater than 1 and about 500, or more. However, it is worth noting that a further addition of detergents, such as those described above, may contribute to the sulfur and/or sulfated ash content of the lubricating oil. These detergents are well known in the art and are commercially available.

### Dispersants

The lubricating oil composition optionally contains dispersants. Typically, the ashless dispersants are nitrogen-containing dispersants formed by reacting alkenyl succinic acid anhydride with an amine. Examples of such dispersants are alkenyl succinimides and succinamides. These dispersants can be further modified by reaction with, for example, boron or ethylene carbonate. Ester-based ashless dispersants derived from long chain hydrocarbon-substituted carboxylic acids and hydroxy compounds may also be employed. Preferred ashless dispersants are those derived from polyisobutenyl succinic anhydride. A large number of dispersants are commercially available.

### Anti-oxidants

Anti-oxidants are used in lubricating oils for inhibition of decomposition processes that occur naturally in lubricating oils as they age or oxidize in the presence of air. These oxidation processes may cause formation of gums, lacquers and sludge resulting in an increase in acidity and viscosity. Examples of useful anti-oxidants are hindered phenols, alkylated and non-alkylated aromatic amines, alkyl or aryl phosphates, esters of thiodicarboxylic acids, salts of carbamic or di-thiophosphoric acids. Molybdenum compounds, such as amine-molybdenum complex compound and molybdenum di-thiocarbamates may also be used as anti-oxidants. However, it should be noted that the addition of molybdenum di-thiocarbamates will further contribute sulfur and sulfated ash to the lubricating oil composition.

### Viscosity Index Improvers

Viscosity index improvers are added to lubricating oil to regulate viscosity changes due to the change in temperature. Some commercially available examples of viscosity index improvers are olefin copolymers, polybutene, polymethacrylates, vinylpyrrolidone and methacrylate copolymers.

### Corrosion inhibitors

Corrosion inhibitors are included in lubricating oils to protect vulnerable metal surfaces. Such corrosion inhibitors are generally used in very small amounts in the range of from 0.02 weight percent to 1.0 weight percent. The corrosion inhibitor should not be one that is itself corrosive to silver and silver plated bearings, such as, metal di-thiophosphates. Examples of corrosion inhibitors that may be used are sulfurized olefin corrosion inhibitor and the co-sulfurized alkenyl ester/alpha olefin corrosion inhibitor. In addition to the materials already described, the lubricating oil composition may also include other additives, such as pour point depressants and anti-foaming agents. The various additive materials or classes of materials herein described are well known materials and can be readily purchased commercially or prepared by known procedures or obvious modification thereof.

### EXAMPLES

The anti-wear additive composition employed in the low sulfur, low sulfated ash and low phosphorus lubricating oil composition were evaluated for their anti-wear performance in formulations prepared as described in Example 1 and Table I below.

### Example 1

Comparative Formulations A and B and Test Formulation C contained an ashless dispersant, an anti-oxidant, a viscosity index improver, a medium overbased alkyl phenate, an anti-wear agent and a foam inhibitor. Base oil was used to make-up a 100 percent of each of Comparative Formulations A and B and Test Formulation C. Comparative Formulations A and B and Test Formulation C are given in more detail in Table I below.

The weight percent calcium concentration based on the total weight of the lubricating oil in each of the Comparative Formulations A and B and Test Formulation C was kept constant, and it is shown in Table II below.

The anti-wear performance of Test Formulation C containing the anti-wear additive composition of the present invention comprising, a calcium salt of a Mannich condensation product, was compared with Comparative Formulation A containing only a mixture of a calcium salt of an alkyl hydroxyaromatic carboxylic acid and a calcium salt of an alkylphenol, and Comparative Formulation B containing a mixture of a calcium I salt of an alkyl hydroxyaromatic carboxylic acid and a calcium salt of an alkylphenol and a calcium salt of a Mannich condensation product.

### Comparative Formulation B contained:

(A) calcium salts of a mixture of:
   (a) a mixture of:
      (i) an alkyl hydroxy benzene carboxylic acid, wherein the alkyl group on the alkyl hydroxy benzene carboxylic acid was a branched chain alkyl group containing 12 carbon atoms, and
      (ii) an alkyl hydroxy benzene carboxylic acid, wherein the alkyl group on the alkyl hydroxy benzene carboxylic acid was a linear chain alkyl group containing 20 carbon atoms to 28 carbon atoms, and
   (b) a mixture of:
      (i) a calcium salt of an alkylphenol, where in the alkyl group on the alkylphenol was a branched chain alkyl group containing 12 carbon atoms, and
      (ii) a calcium salt of an alkylphenol, wherein the alkyl group on the other alkylphenol was a linear chain alkyl group containing 20 carbon atoms to 28 carbon atoms.
         The calcium salt of (a) and (b) were present in a ratio of 3:2, and
(B) a calcium salt of the Mannich condensation product of an alkyl phenol, paraformaldehyde and mono-methyl amine. The Alkyl group on the alkylphenol was a branched chain alkyl group containing 10 carbon atoms to 20 carbon atoms.

Comparative Formulation A contained only (A), shown above in Comparative Formulation B. The calcium salt of (a) and (b) were present in a ratio of 3:2.

Test Formulation C contained only (B), shown above in Comparative Formulation B, the anti-wear additive composition of the present invention.

**Table I**

| **Component** | **Formulation (weight %)** | | |
|---|---|---|---|
| | **Comparative A** | **Comparative B** | **Test C** |
| Base Oil | 92.08 | 91.47 | 90.40 |
| Ashless Dispersant | 3.4 | 3.4 | 3.4 |
| Anti-oxidant | 0.5 | 0.5 | 0.5 |
| Viscosity Index Improver | 0.28 | 0.28 | 0.28 |
| Medium Overbased Phenate | 0.22 | 0.22 | 0.22 |
| Additional Anti-wear Agent | 0.36 | 0.36 | 0.36 |
| Foam Inhibitor | 0.0025 | 0.0025 | 0.0025 |
| (A)* | 3.16 | 2.01 | |
| (B)** | | 1.76 | 4.84 |

Table II below shows the amount of the sulfur, sulfated ash, phosphorus and calcium in Comparative Formulations A and B and Test Formulation C.

**Table II**

| **Component** | **Formulation (weight %)** | | |
|---|---|---|---|
| | **Comparative A** | **Comparative B** | **Test C** |
| Sulfur | 0.0992 | 0.1002 | 0.1007 |
| Sulfated Ash | 1.06 | 1.06 | 1.06 |
| Phosphorus | 0.0378 | 0.0378 | 0.0378 |
| Calcium | 0.296 | 0.296 | 0.296 |

### Example 2

### Modified 4-Ball Test

The anti-wear performance of Test Formulation C was compared to Comparative Formulations A and B was evaluated using a modification of the 4-Ball Test. The modification of the Test involved preaging the samples of Formulations A-C. The Preaging was conducted to allow for the building of a protective layer of the anti-wear additive composition of the present invention and to account for the oxidation decomposition products' impact on an additive's anti-wear performance. Comparative Formulations A and B and Test Formulation C, approximately 10 milliliter samples, were preaged for 2 days at 160°C in the presence of the metal balls. The test was started with a 10 kilogram load, which was increased step-wise to a total of 90 kilograms. Oil temperature at the center of the three fixed balls, torque and displacement of the load lever arm were recorded during the test. A wear index was calculated at the end of the test based on the arm displacement data. This modification of the 4-Ball Test is described in a paper titled Screening Test for Anti-WearAdditives on Modified 4-Ball Test by J. Cazin, P. Tequi and Y. Lesieur, presented at the 10th International Colloquium on Tribology ― Solving Friction and Wear Problems, Technische Akademie Esslingen BRD, January 9-11, 1996, Proceedings Volume 3, 2063-2073.

The data reported were wear index, oil temperature and torque at the end of the test and seizure. The results of the Modified 4-Ball Test are summarized in Table III below.

**Table III**

| Modified 4-Ball Test | Formulation | | |
|---|---|---|---|
| | A | B | C |
| Wear Index* | 276 | 325 | 30 |
| Temperature (°C) | 134 | 131 | 113 |
| Torque (deca-Newton) | 0.246 | 0.243 | 0.159 |
| Seizure | Yes | Yes | No |

| | | | |
|---|---|---|---|
| * Wear Index is obtained by normalizing the actual distance modification on the surface of the balls due to loss of metal because of wear in the Modified 4-Ball Test. The actual distance is measured in micrometers in the Modified 4-Ball Test, but for ease in reporting the numbers obtained in the Test are multiplied by 10. | | | |

The results obtained in the Modified 4-Ball Test summarized above in Table III show that the Test Formulation C containing the anti-wear additive composition used in the present invention comprising a calcium salt of a Mannich condensation product gave better anti-wear performance than Comparative Formulation A containing only a mixture of a calcium salt of an alkyl hydroxyaromatic carboxylic acid and a calcium salt of an alkylphenol or Comparative Formulation B containing both (i) a mixture of a calcium salt of an alkyl hydroxyaromatic carboxylic acid and a calcium salt of an alkylphenol and (ii) a calcium salt of a Mannich condensation product. Table III above shows that in each of the four categories of the data collected Formulation C performed significantly better than either Comparative Formulations A or B.

The data show that Comparative Formulation B, even though it contained some calcium salt of a Mannich condensation product, as in Test Formulation C, Comparative Formulation B did not have anti-wear performance comparable to Test Formulation C. The presence of the mixture of a calcium salt of an alkyl hydroxyaromatic carboxylic acid and a calcium salt of an alkylphenol in Comparative Formulation B, even though Comparative Formulation B contained the calcium salt of a Mannich condensation, appears to have a negative effect on anti-wear performance compared to Test Formulation C, which contained only the calcium salt of a Mannich condensation product of an alkylphenol. This result was unexpected.

## Claims

1. Use of a metal salt of a Mannich condensation product as an anti-wear agent in a low sulfur, low sulfated ash and low phosphorus lubricating oil composition for low emission heavy duty diesel engines, wherein the metal salt of a Mannich condensation product is used in an amount of at least 2 weight percent based on the total weight of the lubricating oil composition, and
wherein:
(a) the sulfur content of the lubricating oil composition is in the range of 0.0 weight percent to 0.4 weight percent based on the total weight of the lubricating oil;
(b) the sulfated ash content of the lubricating oil composition is in the range of 0.2 weight percent to 4.0 weight percent based on the total weight of the lubricating oil; and
(c) the phosphorus content of the lubricating oil composition is in the range of 0.005 weight percent to 0.06 weight percent based on the total weight of the lubricating oil.

2. Use according to claim 1, wherein the concentration of the Mannich condensation product is in the range of from 2 weight percent to 12 weight percent based on the total weight of the lubricating oil composition.

3. Use according to claim 2, wherein the concentration of the Mannich condensation product is in the range of from 3 weight percent to 9 weight percent based on the total weight of the lubricating oil composition.

4. Use according to claim 3, wherein the concentration of the Mannich condensation product is in the range of from 4 weight percent to 7 weight percent based on the total weight of , the lubricating oil composition.

5. Use according to claim 1, wherein in the anti-wear additive composition (b), the Mannich condensation product is a condensation product of an aldehyde having one carbon atom to 20 carbon atoms, a nitrogen base selected from ammonia, a lower alkyl amine, a polyamine and mixtures thereof, and an alkylphenol.

6. Use according to claim 5, wherein the alkyl group on the alkylphenol of the Mannich condensation product is a linear chain or a branched chain alkyl group or mixtures thereof.

7. Use according to claim 6, wherein the alkyl group on the alkylphenol of the Mannich condensation product is a branched chain alkyl group.

8. Use according to claim 5, wherein in the Mannich condensation product the alkyl group on the alkylphenol has from 4 carbon atoms to 60 carbon atoms.

9. Use according to claim 8, wherein the alkyl group on the alkylphenol of the Mannich condensation product has from 6 carbon atoms to 40 carbon atoms.

10. Use according to claim 9, wherein the alkyl group on the alkylphenol of the Mannich condensation product has from 8 carbon atoms to 20 carbon atoms.

11. Use according to claim 5, wherein the alkyl group on the lower alkyl amine has from one carbon atom to 10 carbon atoms and the polyamine has from 2 amine nitrogen atoms to 12 amine nitrogen atoms and 2 carbon atoms to 40 carbon atoms.

12. Use according to claim 11, wherein the nitrogen base for the preparation of the Mannich condensation product is a lower alkyl amine, wherein the alkyl group has one carbon atom to 10 carbon atoms.

13. Use according to claim 12, wherein the lower alkyl amine is an alkyl mono-amine.

14. Use according to claim 11, wherein the polyamine is a mono-alkylene polyamine, polyalkylene polyamine or mixtures thereof.

15. Use according to claim 5, wherein the aldehyde used to prepare the Mannich condensation product is formaldehyde.

16. Use according to claim 5, wherein the aldehyde used to prepare the Mannich condensation product is paraformaldehyde.

17. Use according to claim 5, wherein in the anti-wear additive composition (b) the Mannich condensation product is prepared from an alkylphenol, wherein the alkyl group on the alkylphenol is a branched chain alkyl group having from 8 carbon atoms to 20 carbon atoms, paraformaldehyde and mono-methyl amine.

18. Use according to claim 1, wherein the metal in the metal salt of Mannich condensation product is an alkali metal or an alkaline earth metal.

19. Use according to claim 18, wherein the metal is an alkaline earth metal.

20. Use according to claim 19, wherein the alkaline earth metal is calcium.

21. Use according to claim 21, wherein the sulfur content is in the range of 0.05 weight percent to 0.3 weight percent based on the total weight of the lubricating oil.

22. Use according to claim 21, wherein the sulfur content is in the range of 0.1 weight percent to 0.2 weight percent based on the total weight of the lubricating oil.

23. Use according to claim 21, wherein the sulfated ash content is in the range of 0.3 weight percent to 2.0 weight percent based on the total weight of the lubricating oil.

24. Use according to claim 23, wherein the sulfated ash content is in the range of 0.5 weight percent to 1.2 weight percent based on the total weight of the lubricating oil.

25. Use according to claim 21, wherein the phosphorus content is in the range of 0.015 weight percent to 0.05 weight percent based on the total weight of the lubricating oil.

26. Use according to claim 25, wherein the phosphorus content is in the range of 0.03 weight percent to 0.04 weight

27. Use according to claim 1, wherein the lubricating oil composition further comprises one or more lubricating oil additives selected from detergents, dispersants, anti-oxidants, viscosity index improvers, corrosion inhibitors, anti-wear agents, friction modifiers, pour point depressants and foam inhibitors.

## Patentansprüche

1. Verwendung eines Metallsalzes eines Mannich-Kondensationsprodukts als Verschleißschutzmittel in einer schwefel-, sulfatasche- und phosphorarmen Schmierölzusammensetzung für Hochleistungsdieselmotoren mit geringen Emissionen, wobei das Metallsalz eines Mannich-Kondensationsprodukts in einer Menge von mindestens 2 Gew.-% auf der Basis des Gesamtgewichts der Schmierölzusammensetzung verwendet wird, und wobei
(a) der Schwefelgehalt der Schmierölzusammensetzung im Bereich von 0,0 Gew.-% bis 0,4 Gew.-% ist, auf der Basis des Gesamtgewichts des Schmieröls;
(b) der Sulfataschegehalt der Schmierölzusammensetzung im Bereich von 0,2 Gew.-% bis 4,0 Gew.-% ist, auf der Basis des Gesamtgewichts des Schmieröls; und
(c) des Phosphorgehalt der Schmierölzusammensetzung im Bereich von 0,005 Gew.-% bis 0,06 Gew.-% ist, auf der Basis des Gesamtgewichts des Schmieröls.

2. Verwendung gemäß Anspruch 1, wobei die Konzentration des Mannich-Kondensationsprodukts im Bereich von 2 Gew.-% bis 12 Gew.-% auf der Basis des Gesamtgewichts der Schmierölzusammensetzung ist.

3. Verwendung gemäß Anspruch 2, wobei die Konzentration des Mannich-Kondensationsprodukts im Bereich von 3 Gew.-% bis 9 Gew.-% auf der Basis des Gesamtgewichts der Schmierölzusammensetzung ist.

4. Verwendung gemäß Anspruch 3, wobei die Konzentration des Mannich-Kondensationsprodukts im Bereich von 4 Gew.-% bis 7 Gew.-% auf der Basis des Gesamtgewichts der Schmierölzusammensetzung ist.

5. Verwendung gemäß Anspruch 1, wobei in der Verschleißschutzzusatzzusammensetzung (b) das Mannich-Kondensationsprodukt ein Kondensationsprodukt eines Aldehyds mit einem Kohlenstoffatom bis 20 Kohlenstoffatomen, einer Stickstoffbase, ausgewählt aus Ammoniak, einem niederen Alkylamin, einem Polyamin oder Gemischen davon, und eines Alkylphenols ist.

6. Verwendung gemäß Anspruch 5, wobei die Alkylgruppe auf dem Alkylphenol des Mannich-Kondensationsprodukts eine Alkylgruppe mit linearer Kette oder verzweigter Kette oder Gemische davon ist.

7. Verwendung gemäß Anspruch 6, wobei die Alkylgruppe auf dem Alkylphenol des Mannich-Kondensationsprodukts eine Alkylgruppe mit verzweigter Kette ist.

8. Verwendung gemäß Anspruch 5, wobei im Mannich-Kondensationsprodukt die Alkylgruppe auf dem Alkylphenol von 4 Kohlenstoffatomen bis 60 Kohlenstoffatomen hat.

9. Verwendung gemäß Anspruch 8, wobei die Alkylgruppe auf dem Alkylphenol des Mannich-Kondensationsprodukts von 6 Kohlenstoffatomen bis 40 Kohlenstoffatomen hat.

10. Verwendung gemäß Anspruch 9, wobei die Alkylgruppe auf dem Alkylphenol des Mannich-Kondensationsprodukts von 8 Kohlenstoffatomen bis 20 Kohlenstoffatomen hat.

11. Verwendung gemäß Anspruch 5, wobei die Alkylgruppe auf dem niederen Alkylamin von einem Kohlenstoffatom bis 10 Kohlenstoffatomen hat und das Polyamin von 2 Aminstickstoffatome bis 12 Aminstickstoffatome und 2 Kohlenstoffatome bis 40 Kohlenstoffatome.

12. Verwendung gemäß Anspruch 11, wobei die Stickstoffbase für die Herstellung des Mannich-Kondensationsprodukts ein niederes Alkylamin ist, wobei die Alkylgruppe ein Kohlenstoffatom bis 10 Kohlenstoffatome hat.

13. Verwendung gemäß Anspruch 12, wobei das niedere Alkylamin ein Alkylmonoamin ist.

14. Verwendung gemäß Anspruch 11, wobei das Polyamin ein Monoalkylenpolyamin, ein Polyalkylenpolyamin oder Gemische davon ist.

15. Verwendung gemäß Anspruch 5, wobei das für die Herstellung des Mannich-Kondensationsprodukts verwendete Aldehyd Formaldehyd ist.

16. Verwendung gemäß Anspruch 5, wobei das für die Herstellung des Mannich-Kondensationsprodukts verwendete Aldehyd Paraformaldehyd ist.

17. Verwendung gemäß Anspruch 5, wobei in der Verschleißschutzzusatzzusammensetzung (b) das Mannich-Kondensationsprodukt hergestellt wird aus einem Alkylphenol, wobei die Alkylgruppe auf dem Alkylphenol eine verzweigte Alkylkette ist mit von 8 Kohlenstoffatomen bis 20 Kohlenstoffatomen, aus Paraformaldehyd und aus Monomethylamin.

18. Verwendung gemäß Anspruch 1, wobei das Metall im Metallsalz des Mannich-Kondensationsprodukts ein Alkalimetall oder ein Alkalierdmetall ist.

19. Verwendung gemäß Anspruch 18, wobei das Metall ein Alkalierdmetall ist.

20. Verwendung gemäß Anspruch 19, wobei das Alkalierdmetall Calcium ist.

21. Verwendung gemäß Anspruch 1, wobei der Schwefelgehalt im Bereich von 0,05 Gew.-% bis 0,3 Gew.-% ist, auf der Basis des Gesamtgewichts des Schmieröls.

22. Verwendung gemäß Anspruch 21, wobei der Schwefelgehalt im Bereich von 0,1 Gew.-% bis 0,2 Gew.-% ist, auf der Basis des Gesamtgewichts des Schmieröls.

23. Verwendung gemäß Anspruch 1, wobei der Sulfataschegehalt im Bereich von 0,3 Gew.-% bis 2,0 Gew.-% ist, auf der Basis des Gesamtgewichts des Schmieröls.

24. Verwendung gemäß Anspruch 23, wobei der Sulfataschegehalt im Bereich von 0,5 Gew.-% bis 1,2 Gew.-% ist, auf der Basis des Gesamtgewichts des Schmieröls.

25. Verwendung gemäß Anspruch 1, wobei der Phosphorgehalt im Bereich von 0,015 Gew.-% bis 0,05 Gew.-% ist, auf der Basis des Gesamtgewichts des Schmieröls.

26. Verwendung gemäß Anspruch 25, wobei der Phosphorgehalt im Bereich von 0,03 Gew.-% bis 0,04 Gew.-% ist, auf der Basis des Gesamtgewichts des Schmieröls.

27. Verwendung gemäß Anspruch 1, wobei die Schmierölzusammensetzung zudem umfasst ein oder mehrere Schmierölzusatzmittel, ausgewählt aus Detergenzien, Dispergiermitteln, Antioxidationsmitteln, Viskositätsindexverbesserern, Korrosionsverringerern, Antiverschleißmitteln, Reibungsmodifizierern, Pourpointverringerern und Schauminhibitoren.

## Revendications

1. Utilisation d'un sel métallique d'un produit de condensation Mannich comme agent anti-usure dans une composition d'huile lubrifiante à faible teneur en soufre, en cendres sulfatées et en phosphore pour des moteurs diesel de haute performance à émissions réduites, le sel métallique d'un produit de condensation Mannich étant utilisé en une quantité d'au moins 2 pourcent en poids sur la base du poids total de la composition d'huile lubrifiante, et dans laquelle :
(a) la teneur en soufre de la composition d'huile lubrifiante est dans l'intervalle de 0,0 pourcent en poids à 0,4 pourcent en poids sur la base du poids total de l'huile lubrifiante ;
(b) la teneur en cendres sulfatées de la composition d'huile lubrifiante est dans l'intervalle de 0,2 pourcent en poids à 4,0 pourcent en poids sur la base du poids total de l'huile lubrifiante ; et
(c) la teneur en phosphore de la composition d'huile lubrifiante est dans l'intervalle de 0,005 pourcent en poids à 0,06 pourcent en poids sur la base du poids total de l'huile lubrifiante.

2. Utilisation selon la revendication 1, dans laquelle la concentration du produit de condensation Mannich est dans l'intervalle entre 2 pourcent en poids et 12 pourcent en poids sur la base du poids total de la composition d'huile lubrifiante.

3. Utilisation selon la revendication 2, dans laquelle la concentration du produit de condensation Mannich est dans l'intervalle entre 3 pourcent en poids et 9 pourcent en poids sur la base du poids total de la composition d'huile lubrifiante.

4. Utilisation selon la revendication 3, dans laquelle la concentration du produit de condensation Mannich est dans l'intervalle entre 4 pourcent en poids et 7 pourcent en poids sur la base du poids total de la composition d'huile lubrifiante.

5. Utilisation selon la revendication 1, dans laquelle dans la composition d'additif anti-usure (b), le produit de condensation Mannich est un produit de condensation d'un aldéhyde ayant un atome de carbone à 20 atomes de carbone, d'une base azotée sélectionnée parmi l'ammoniac, une alkylamine légère, une polyamine et leurs mélanges, et d'un alcoylphénol.

6. Utilisation selon la revendication 5, dans laquelle le groupe alkyle sur l'alcoylphénol du produit de condensation Mannich est un groupe alkyle à chaine linéaire ou un groupe alkyle à chaine branchée ou un de leurs mélanges.

7. Utilisation selon la revendication 6, dans laquelle le groupe alkyle sur l'alcoylphénol du produit de condensation Mannich est un groupe alkyle à chaine branchée.

8. Utilisation selon la revendication 5, dans laquelle dans le produit de condensation Mannich, le groupe alkyle sur l'alcoylphénol a entre 4 atomes de carbone et 60 atomes de carbone.

9. Utilisation selon la revendication 8, dans laquelle le groupe alkyle sur l'alcoylphénol dans le produit de condensation Mannich a entre 6 atomes de carbone et 40 atomes de carbone.

10. Utilisation selon la revendication 9, dans laquelle le groupe alkyle sur l'alcoylphénol dans le produit de condensation Mannich a entre 8 atomes de carbone et 20 atomes de carbone.

11. Utilisation selon la revendication 5, dans laquelle le groupe alkyle sur l'alkylamine légère a entre un atome de carbone et 10 atomes de carbone et la polyamine a entre 2 atomes d'azote d'amine et 12 atomes d'azote d'amine et entre 2 atomes de carbone et 40 atomes de carbone.

12. Utilisation selon la revendication 11, dans laquelle la base azotée pour la préparation du produit de condensation Mannich est une alkylamine légère, le groupe alkyle ayant entre un atome de carbone et 10 atomes de carbone.

13. Utilisation selon la revendication 12, dans laquelle l'alkylamine légère est une alkylemonoamine.

14. Utilisation selon la revendication 11, dans laquelle la polyamine est une monoalcylène-polyamine, une polyalcylène-polyamine ou leurs mélanges.

15. Utilisation selon la revendication 5, dans laquelle l'aldéhyde utilisé pour préparer le produit de condensation Mannich est le formaldéhyde.

16. Utilisation selon la revendication 5, dans laquelle l'aldéhyde utilisé pour préparer le produit de condensation Mannich est le paraformaldéhyde.

17. Utilisation selon la revendication 5, dans laquelle dans la composition d'additif anti-usure (b), le produit de condensation Mannich est préparé à partir d'un alcoylphénol, le groupe alkyle dans l'alcoylphénol étant un groupe alkyle à chaine branchée ayant entre 8 atomes de carbone et 20 atomes de carbone, du paraformaldéhyde et d'une monométhylamine.

18. Utilisation selon la revendication 1, dans laquelle le métal dans le sel métallique d'un produit de condensation Mannich est un métal alcalin ou un métal alcalino-terreux.

19. Utilisation selon la revendication 18, dans laquelle le métal dans le sel métallique d'un produit de condensation Mannich est un métal alcalino-terreux.

20. Utilisation selon la revendication 19, dans laquelle le métal alcalino-terreux est le calcium.

21. Utilisation selon la revendication 1, dans laquelle la teneur en soufre est dans l'intervalle de 0,05 pourcent en poids à 0,3 pourcent en poids sur la base du poids total de l'huile lubrifiante.

22. Utilisation selon la revendication 21, dans laquelle la teneur en soufre est dans l'intervalle de 0,1 pourcent en poids à 0,2 pourcent en poids sur la base du poids total de l'huile lubrifiante.

23. Utilisation selon la revendication 1, dans laquelle la teneur en cendres sulfatées est dans l'intervalle de 0,3 pourcent en poids à 2,0 pourcent en poids sur la base du poids total de l'huile lubrifiante.

24. Utilisation selon la revendication 23, dans laquelle la teneur en cendres sulfatées est dans l'intervalle de 0,5 pourcent en poids à 1,2 pourcent en poids sur la base du poids total de l'huile lubrifiante.

25. Utilisation selon la revendication 1, dans laquelle la teneur en phosphore est dans l'intervalle de 0,015 pourcent en poids à 0,05 pourcent en poids sur la base du poids total de l'huile lubrifiante.

26. Utilisation selon la revendication 25, dans laquelle la teneur en phosphore est dans l'intervalle de 0,03 pourcent en poids à 0,04 pourcent en poids sur la base du poids total de l'huile lubrifiante.

27. Utilisation selon la revendication 1, dans laquelle la composition d'huile lubrifiante contient en plus un ou plusieurs additifs pour huile lubrifiante, sélectionnés parmi détergents, dispersants, antioxydants, améliorants d'indice de viscosité, inhibiteurs de corrosion, agents anti-usure, modificateurs de friction, abaisseurs de point d'écoulement et agents antimousse.
